

[54] PROCESS FOR MAKING A NOVEL COPPER  
BASE ALLOY

[75] Inventors: **Jacob Crane**, Woodbridge; **Sam Friedman**, Hamden; **Michael Joseph Pryor**, Woodbridge, all of Conn.

[73] Assignee: **Olin Corporation**, New Haven, Conn.

[22] Filed: **Sept. 20, 1973**

[21] Appl. No.: **399,073**

**Related U.S. Application Data**

[63] Continuation-in-part of Ser. No. 268,485, July 3, 1972, Pat. No. 3,816,109.

[52] U.S. Cl. .... **148/2**, 148/11.5 R, 148/12.7,  
148/32, 148/32.5

[51] Int. Cl. .... **C22f 1/08**

[58] Field of Search ..... 148/2, 3, 11.5 R, 12.7,  
148/32, 32.5, 13.2, 160; 75/153, 157.5

[56] **References Cited**

UNITED STATES PATENTS

|           |        |             |          |
|-----------|--------|-------------|----------|
| 1,723,922 | 8/1929 | Corson..... | 75/153   |
| 1,959,509 | 5/1934 | Tour .....  | 75/157.5 |
| 2,126,827 | 8/1938 | Smith.....  | 148/11.5 |
| 2,147,844 | 2/1939 | Kelly.....  | 75/153   |

|           |        |                |            |
|-----------|--------|----------------|------------|
| 2,155,406 | 4/1939 | Crampton ..... | 75/157.5 X |
| 2,169,188 | 8/1939 | Kelly.....     | 75/157.5 X |
| 2,295,180 | 9/1942 | Mitchell.....  | 75/157.5   |

Primary Examiner—C. Lovell

Attorney, Agent, or Firm—David A. Jackson; Robert H. Bachman

[57] **ABSTRACT**

A method of preparing a copper alloy is disclosed which comprises providing in the alloy about 0.8 – 2.3% iron and about 0.3 – 1.7% cobalt, such that the amount of iron plus cobalt ranges from about 1.5 – 2.5%, from about 5 – 13% zinc, balance essentially copper. The alloy is hot rolled at a temperature of at least 500°C, and cold rolled by a process which includes conducting at least one interanneal between successive cold reductions. The interanneal is conducted at temperatures ranging from about 400 to 600°C for a period of at least 15 minutes. Processing may also include a final anneal at a temperature of from 350 to 600°C conducted for at least 15 minutes. The novel alloy of this invention possesses a combination of strength and electrical conductivity which makes it a suitable replacement for the C.D.A. 400 series tin-brass alloys.

**8 Claims, 1 Drawing Figure**

PATENTED DEC 3 1974

3,852,121



PROCESS FOR MAKING A NOVEL COPPER BASE  
ALLOY

CROSS REFERENCE TO RELATED APPLICATION

5

The present application is a continuation-in-part of copending application Ser. No. 268,485, by Jacob Crane, Sam Friedman and Michael J. Pryor for COPPER BASE ALLOY, filed July 3, 1972, now U.S. Pat. No. 3,816,109.

BACKGROUND OF THE INVENTION

This invention provides for the methods of processing a copper base alloy disclosed in our co-pending application Ser. No. 268,485. The novel alloys disclosed therein were found to possess a unique combination of strength and electrical conductivity which makes them suitable for use in structural electrical components. The alloy possesses sufficient ductility to be formed into intricate parts such as electrical receptacles. Since such parts are used in a variety of environments and are in a highly stressed condition, stress corrosion is highly important.

Tin-brasses, namely, the C.D.A. 400 series alloys are commonly used for this type of application since they combine the above described properties. In general, the electrical conductivity of these 400 series alloys ranges from 28% IACS for C.D.A. Alloy 425 which is the strongest of the series, to 41% IACS for C.D.A. Alloy 405 which possesses the lowest strength of the series. Various of these alloys, particularly those containing higher tin concentrations, are difficult to manufacture, particularly with regard to casting and hot rollability.

SUMMARY OF THE INVENTION

In accordance with this invention, a copper base alloy containing about 0.8 - 2.3% iron and about 0.3 - 40 1.7% cobalt wherein the amount of iron plus cobalt ranges from about 1.5 to 2.5%, from about 5 to 13% zinc, balance essentially copper, is prepared by a process which comprises hot rolling at a temperature of at least 500°C, and cold rolling the alloy to a cross sectional area reduction of at least 50%, said cold rolling including one or more cold reduction steps followed by one or more interanneals conducted at a temperature of from 400 to 600°C for at least 15 minutes.

The novel alloys processed in accordance with this invention provide electrical conductivity that is superior to those of the 400 series tin-brasses at a comparable strength to limiting bend radius ratio; or at comparable conductivity, they provide superior strength to limiting bend radius ratio.

Accordingly, it is a principal object of this invention to provide a method of processing a copper base alloy containing iron, cobalt and zinc within specific ranges which results in an alloy possessing an improved combination of strength and electrical conductivity.

It is a further object of this invention to provide a method as aforesaid which provides alloys with properties which make them suitable substitutes for the tin-brasses.

Other objects and advantages will become apparent to those skilled in the art from the detailed description which follows.

BRIEF DESCRIPTION OF THE DRAWING

The accompanying FIGURE is a graph of tensile strength (KSI) and electrical conductivity (% IACS) measured from alloy samples annealed at various temperatures for 1 hour.

DETAILED DESCRIPTION OF THE PREFERRED  
EMBODIMENTS

In accordance with this invention, a method of processing a novel copper base alloy is disclosed which achieves a unique combination of strength and electrical conductivity in the alloy that is superior to the tin-brasses, and is less difficult to practice.

The method of this invention initially comprises providing a copper base alloy containing from about 0.8 to about 2.3% iron and from about 0.3 to about 1.7% cobalt such that the amount of iron plus cobalt ranges from about 1.5 to about 2.5%, from about 5 to about 20 13% zinc, balance essentially copper. Impurities may be present in amounts which do not adversely affect the properties of the above alloy.

Impurities at the following levels separately or in combination do not adversely affect the casting or hot and cold rolling characteristics of the alloy. Thus, the alloy may contain up to about 0.03% phosphorous, up to about 0.03% lead, up to about 0.05% tin, up to about 0.05% nickel, up to about 0.10% manganese, up to about 0.10% aluminum, up to about 0.05% silver and up to about 0.10% silicon. It is preferred that the maximum total impurities be limited to less than 0.2% to minimize adverse affect on the properties of the alloys.

In additional features and advantages of the alloy are fully set forth in co-pending application Ser. No. 268,485, now U.S. Pat. No. 3,816,109, which is incorporated herein by reference.

The alloys of this invention may be prepared in accordance with the following practice.

*Melting and Casting:* The copper is melted, the iron and cobalt are added to the melt and it is then heated to about 1300°C and held at that temperature until the iron and cobalt are thoroughly dissolved. The temperature of the melt is reduced to about 1200°C and the zinc is then added. The temperature at which the molten alloy is poured should be sufficiently high to assure a temperature no lower than about 1175°C at the mold, in order to avoid the formation of coarse primary particles rich in iron and cobalt. Other casting parameters are in accordance with conventional practice in the art. The choice of casting method is not critical, as the alloy can be either static cast or direct chill (DC) cast.

*Hot Rolling:* The case alloy is soaked at a temperature of from about 800 to about 1000°C and preferably from about 900 to about 950°C. Soak time is not critical and may be varied as desired from a few minutes up to an hour or more. The pass schedule may, likewise, be set as desired. Pass speed is variable, as reduction can be achieved in a matter of minutes, or could be extended to hours' duration depending upon the particular sequence employed by the artisan. Thus, for example, reduction of from 5 inches to 0.40 inches would take of the order of minutes if done at one time, but could take hours if the alloy is permitted to cool off between passes. Pass temperature, however, should preferably be above about 500°C but below the melting temperature of the alloy. It would be possible to permit

the alloy to cool below 500°C between passes, however, such practice is uneconomical as extensive re-heating would be necessary. It is, therefore, preferable to maintain the alloy at a temperature above 500°C throughout the entire hot rolling step. The alloys of this invention have better than 75% cold rollability if the hot rolling operation is completed above 500°C. Finishing temperatures of lower than 500°C may be employed if some subsequent loss in cold rollability is acceptable.

*Cold Rolling:* The hot rolled alloy is then cold rolled. As previously noted, cold reductions in excess of 75% can be achieved if the hot rolling finishing temperature is above 500°C. Cold rolling to any specified finished gage may require interannealing. After suitable annealing, the alloy still possesses cold rollability in excess of 75% reduction. Where the optimum combination of strength and formability of a temper rolled product is desired, a minimum of 50% reduction should be attained prior to the last interanneal. Thus, if only one interanneal is employed between two cold reductions, the alloy should be cold rolled to at least a 50% reduction in the first cold reduction, whereas if a series of cold reductions and interanneals are employed, only the cold reduction conducted prior to the last interanneal must achieve the required minimum of at least 50% reduction.

*Annealing:* Annealing for softening can be performed either by bell or strip annealing. The choice of bell annealing versus strip annealing is predicated upon desired electrical conductivity. Where maximum conductivity is required, bell annealing is preferred.

As noted earlier, for the purpose of obtaining improved strength in the cold worked condition, at least one interanneal is conducted between successive cold reductions. The interanneal should be carried out for a period of at least 15 minutes at temperatures of from about 400 to about 600°C. Preferably the interanneal is conducted at a temperature ranging from about 450 to about 550°C for from about 1 to about 16 hours. It has been found that this latter schedule yields more favorable results when bell annealing is conducted. At least one interanneal is required to achieve a strength potential within the scope of this invention, however, multiple interanneals can be used between cold reductions as desired.

It has been observed that the alloy prepared by this process possesses an unexpectedly improved strength and conductivity over alloys prepared by a process which employs only cold reduction. These findings are illustrated by the results of Example I which follows.

#### EXAMPLE I

An alloy was prepared having the following composition (in weight percent): Cu - 11.3% Zn - 1.6% Fe - 0.5% Co. The alloy was melted at 1300°C and DC cast at 1190°C. The cast alloy was hot rolled from 5 inches thick to 0.40 inch thick at a starting temperature of 960°C and a finishing temperature of 690°C, and was then coil milled to 0.360 inch thick to produce a clean surface. The hot rolled plate was then processed variously as follows:

##### PROCESS A:

cold rolled 60%

##### PROCESS B:

cold rolled 77%

##### PROCESS C:

cold rolled 0.080" gage;  
bell annealed at 540°C-1 hr;  
cold rolled 50%.

##### PROCESS D:

cold rolled to 0.080" gage;  
bell annealed at 540°C-1 hr;  
cold rolled 61%.

##### PROCESS E:

cold rolled to 0.140" gage;  
bell annealed at 540°C-1 hr;  
cold rolled to 0.060" gage;  
bell annealed at 525°C-1 hr;  
cold rolled 50%.

##### PROCESS F:

cold rolled to 0.140" gage;  
bell annealed at 540°C-1 hr;  
cold rolled to 0.060" gage;  
bell annealed at 525°C-1 hr;  
cold rolled 75%.

The tensile strengths obtained as a result of the following processes are shown in Table I, below.

TABLE I

| Process | % Final Reduction | UTS (KSI) | Number of In-Process Anneals |
|---------|-------------------|-----------|------------------------------|
| A       | 60                | 83        | None                         |
| B       | 77                | 88        | None                         |
| C       | 50                | 91        | 1                            |
| D       | 61                | 96        | 1                            |
| E       | 50                | 90        | 2                            |
| F       | 75                | 98        | 2                            |

Referring to the results of Table I, it is noted that the alloy prepared by Process D, in accordance with this invention, which involved 61% cold reduction and one interanneal, possessed an ultimate tensile strength of 96 KSI, whereas the same alloy prepared by Process A, which involved a 60% cold reduction but which omitted the interannealing step, possessed an ultimate tensile strength of only 83 KSI. Likewise, the alloy prepared by Process F which involved a 75% cold reduction and two interanneals, possessed an ultimate tensile strength of 98 KSI, whereas the same alloy prepared by Process B, which involved a 77% cold reduction with no interanneals possessed an ultimate tensile strength of 88 KSI. It is clear from this comparison that the employment of at least one interanneal provides a significant improvement in the tensile strength of the cold rolled alloys which cannot be duplicated simply by increased cold reduction only.

It has also been found that the bend properties of an alloy at a given strength level are affected by the interannealing parameters employed. Thus, variation of either one or both of the temperature and duration of the interanneal can result in alloys which have different minimum bend radii. This relationship is illustrated in Example II, below.

#### EXAMPLE II

Two alloys of composition (in weight percent) Cu - 12.2% Zn - 1.7% Fe - 0.6% Co, and Cu - 10.0% Zn - 1.7% Fe - 0.5% Co, respectively, were melted at 1300°C and Durville cast at 1175°C. The alloys were hot rolled from 1 1/4 inches thick to approximately 0.35 inch thick at starting temperatures of about 950°C and a finishing temperature of about 625°C; surface milled to produce a clear surface; cold rolled to 0.080 inch

gage; annealed at various temperatures for various times; cold rolled to 0.020 inch gage.

The tensile strength and minimum bend radius of the 0.020 inch gage metal measured with the bend axis parallel to the rolling direction ("bad way" bend), and 90° to the rolling direction ("good way" bend) are shown in Table II, below.

TABLE II

| 0.080" Gage<br>INTERANNEAL<br>Temp., (°C) | 0.080" Gage<br>INTERAN-<br>NEAL<br>Time, (Hrs.) | UTS<br>(KSI) | 0.020" Gage<br>MIN. BEND RADIUS, 64th |         |
|-------------------------------------------|-------------------------------------------------|--------------|---------------------------------------|---------|
|                                           |                                                 |              | Good Way                              | Bad Way |
| <b>Cu-12.2% Zn-1.7% Fe-0.6% Co</b>        |                                                 |              |                                       |         |
| 400                                       | 4                                               | 101          | 3                                     | 16      |
| 400                                       | 16                                              | 101          | 2                                     | 12      |
| 450                                       | 1                                               | 100          | 2                                     | 16      |
| 450                                       | 4                                               | 100          | 3                                     | 12      |
| 500                                       | 1                                               | 101          | 3                                     | 12      |
| 500                                       | 4                                               | 101          | 3                                     | 12      |
| 500                                       | 16                                              | 100          | 2                                     | 12      |
| <b>Cu-10.0% Zn-1.7% Fe-0.5% Co</b>        |                                                 |              |                                       |         |
| 450                                       | 1                                               | 96           | 2                                     | 12      |
| 450                                       | 4                                               | 97           | 2                                     | 10      |
| 500                                       | 1                                               | 98           | 2                                     | 10      |
| 500                                       | 4                                               | 96           | 2                                     | 8       |
| 500                                       | 16                                              | 96           | 2                                     | 8       |

For final gage annealing of cold metal, a range of about 350 to about 600°C is desirable. The annealing temperature within this range may be varied depending upon the strength and electrical conductivity properties desired in the alloy. Thus, for maximum conductivity, annealing is preferably conducted in the range of about 350 to about 450°C, whereas if major softening is desired, annealing in the range of about 400 to about 600°C is preferred. Final gage annealing is normally conducted for at least 15 minutes, and is preferably conducted for a period of from about 1 to about 8 hours. The employment of the final gage anneal in the above-described manner is illustrated in Example III, below.

### EXAMPLE III

An alloy of composition Cu - 11.9% Zn - 1.5% Fe - 0.5% Co was melted at 1300°C and DC cast at 1175°C. The alloy was then hot rolled from 3 inches thick to approximately 0.40 inch thick at a starting temperature of 975°C and a finishing temperature of about 400°C. The hot rolled alloy was then surface milled to product a clean surface; cold rolled to 0.080 inch gage; annealed at 500°C for 1 hour; and cold rolled to 0.020 inch final gage. The samples thus prepared were then finally annealed at various temperatures for 1 hour.

The electrical conductivities and tensile strengths of the variously annealed samples were measured, and the resulting data is presented in the graph in the accompanying FIGURE, wherein electrical conductivity and tensile strength have been plotted as functions of annealing temperature.

Referring to the FIGURE, it can be seen that, in the range of 350 - 450°C, an optimum combination of strength and conductivity is attained that results in alloys suited for a wide variety of electrical uses. Also, as stated earlier, temperatures of between 350 and 450°C yield maximum conductivity, as conductivities of between about 35 to about 37% IACS are shown. Likewise, if further softening is desirable, temperatures ranging from 400 to 600°C could be employed with only a minor loss of conductivity, i.e. levels of 33 to

31% IACS. Thus, as shown in the FIGURE, the preparation of a finally annealed alloy possessing a particular combination of tensile strength and conductivity can be controlled by the careful selection of the final annealing temperature.

Referring again to the FIGURE, the strength and conductivity of the as-rolled alloy were also measured

and plotted. The resulting data demonstrates that high tensile strength and acceptable conductivity are attainable by the employment of an interannealing step during the cold rolling of the alloy, in accordance with the process of this invention.

When cast in accordance with the methods of this invention, the copper alloy possesses a microstructure characterized by an average grain diameter in the order of 0.1 mm and an iron-cobalt rich phase with a particle size in the order of 0.01 mm, more or less uniformly distributed throughout the copper matrix. The said particles tend to have angular boundaries, with the exception of some particles which may exhibit dendritic form with short dentrite arms.

The microstructure resulting from annealing the cold worked metal in the temperature range of about 450 to about 650°C is characterized by fine, equiaxed grains which resist significant growth. The average recrystallized grain diameter remains less than 0.010 mm in diameter over the aforementioned temperature range. The approximate equiaxed iron-cobalt rich particles that exist in the cast structure, are elongated in the rolling direction, the extent of the elongation being dependent upon the total percent reduction of the main body of metal.

The alloys prepared by the process of this invention have particular application in structural electrical components such as electrical contacts, electrical receptacles, electrical connectors and the like.

All of the compositions specified in this application by percentage are given in percentage by weight.

This invention may be employed in other forms or carried out in other ways without departing from the spirit or essential characteristics thereof. The present embodiment is therefore to be considered as in all respects illustrative and not restrictive, the scope of the invention being indicated by the appended claims, and all changes which come within the meaning and range of equivalency are intended to be embraced therein.

What is claimed is:

1. A method of preparing copper alloys consisting essentially of about 0.8-2.3% iron and about 0.3-1.7%

cobalt, such that the amount of iron plus cobalt ranges from about 1.5 to 2.5%, from 5 to 13% zinc and the balance essentially copper, to provide improved strength, bend properties, and electrical properties which comprises:

- a. hot rolling the alloy at a temperature of at least 500°C, but below its melting temperature; and
  - b. cold rolling to at least 50% cold reduction wherein said cold rolling includes successive cold reductions and at least one interanneal conducted therebetween at temperatures ranging from about 400 to 600°C for a period of at least 15 minutes.
2. The method of claim 1 wherein the cold reduction conducted prior to the last interanneal yields a cross sectional area reduction of at least 50%.
3. The method of claim 1 wherein said interanneal is conducted at temperatures ranging from about 450 to

500°C for from 1 to 4 hours.

4. The method of claim 1 wherein said alloy is melted at a temperature of from about 1200 to 1300°C, and cast at a temperature such that the resultant mold temperature is at least 1175°C.
5. The method of claim 1 wherein, prior to hot rolling, the alloy is soaked at a temperature of from 800 to 1000°C for a period of up to 1 hour.
6. The method of claim 5 wherein said alloy is soaked at a temperature of from 900 to 950°C.
7. The method of claim 1 wherein the cold rolled alloy is finally annealed at a temperature of 350 – 600°C for at least 15 minutes.
8. The method of claim 7 wherein the final anneal is conducted at a temperature of from 350 to 450°C for from 1 to 8 hours.

\* \* \* \* \*

20

25

30

35

40

45

50

55

60

65

UNITED STATES PATENT OFFICE  
CERTIFICATE OF CORRECTION

Patent No. 3,852,121 Dated December 3, 1974

Inventor(s) Jacob Crane, Sam Friedman and Michael J. Pryor

It is certified that error appears in the above-identified patent and that said Letters Patent are hereby corrected as shown below:

In Column 8, corresponding to Claim 3, line 1, after "to", please delete the number "500°C" and insert in its place -- 550°C --.

Signed and sealed this 11th day of March 1975.

(SEAL)

Attest:

RUTH C. MASON  
Attesting Officer

C. MARSHALL DANN  
Commissioner of Patents  
and Trademarks